

FIP8309

XR

1,573,200

CAJUN U.S. Patented Feb. 16, 1926.

8-9

1,573,200

## UNITED STATES PATENT OFFICE.

HYMAN STEIN, OF ARVERNE, WILLIAM E. AUSTIN, OF NEW YORK, AND IRVING LIEBOWITZ, OF BROOKLYN, NEW YORK, ASSIGNORS TO STEIN FUR DYEING CO., INC., OF NEW YORK, N. Y., A CORPORATION OF NEW YORK.

## PROCESS OF BLEACHING AND DYEING FURS AND THE LIKE.

No Drawing.

Application filed May 3, 1924. Serial No. 710,829.

To all whom it may concern:

Be it known that we, HYMAN STEIN, WILLIAM E. AUSTIN, and IRVING LIEBOWITZ, citizens of the United States, residing, respectively, in Arverne, Queens County, city and State of New York, in the borough of the Bronx, Bronx County, city and State of New York, and in the borough of Brooklyn, Kings County, city and State of New York, 10 have invented an Improvement in Processes of Bleaching and Dyeing Furs and the like, of which the following is a specification.

Our present invention relates to methods of bleaching and thereafter dyeing fibres, particularly animal fibres, especially fur skins and the like, and aims to devise methods of the general character specified above whereby articles of the classes mentioned, especially dark colored fur skins and other 20 fibrous products, particularly of animal origin, may be bleached or decolorized in a simple, convenient, economical and expeditious manner, and without impairing the strength or texture of the articles bleached 25 in accordance with the principles of the present invention, which articles may, after the bleaching operation, be simply conveniently, economically and expeditiously dyed so as to yield a high grade product characterized by unusual strength and remarkably fine texture, and by a very attractive appearance which recommends itself highly to purchasers of such articles and thus gives the articles made by the methods of the present invention a wide and profitable market.

While not limited thereto, our present invention finds particularly successful application in the bleaching or decolorizing, and subsequent dyeing, of dark colored fur skins 40 which may, by means of the method of the present invention, be bleached or decolorized without impairing the strength or texture of either the leather or the hair of such fur skins, and which may thereafter be dyed the same colors as can at present be applied only to white or very light colored furs, which white or light colored furs are, as well known to those skilled in the art to which the present invention relates, comparatively 45 expensive; the combined bleaching or decolorizing and subsequent dyeing operations requiring, under the conditions of the present invention, only as much time, in the

average case, as the ordinary fur dyeing process alone.

In the accompanying specification we shall describe an illustrative embodiment of the method of the present invention as applied more particularly to the bleaching or decolorizing and the subsequent dyeing of fur skins or the like. It is, however, to be clearly understood that our invention is not limited to the specific embodiments thereof herein described for purposes of illustration only, and that the process may be applied with almost equal success to the bleaching or decolorizing and subsequent dyeing of other fibrous products, particularly of animal origin, than the fur skins here specifically described. It may here also be stated that the bleached or decolorized, and the subsequently dyed, products, while described herein as the result of practicing the process herein described and claimed, are themselves described and claimed in another copending application filed by us of even date herewith and entitled "Bleached and dyed furs and the like," Serial No. 710,830.

Before describing in detail the aforesaid illustrative embodiment of the method of the present invention, it may be desirable briefly to point out the defects and disadvantages of the prior art to which the present invention relates. Hitherto, in attempting to bleach or decolorize and thereafter to dye dark colored fur skins and the like, in an effort to convert the same to a light colored skin, so that the same might be dyed a light color in the same manner as the natural white or light colored skins might be dyed, it has been customary to use a comparatively powerful bleaching agent in order to bleach or decolorize the dark colored fur skins or the like. For example, it has hitherto been proposed to use such powerful bleaching agents as hydrogen peroxide, hypochlorites, permanganates, sulphites, hydrosulphites, and the like. By the use of such powerful bleaching agents it has been impossible to bleach or decolorize dark colored fur skins or the like without seriously weakening, or even destroying, the leather and without weakening or even seriously impairing the natural strength and texture of the hair of such fur skins to such a degree as to render the skins unfit for further use. Further-

55

60

65

70

75

80

85

90

95

100

105

TREATMENT & CHEMICAL MODIFI-  
CATION OF TEXTILES & FIBERS,

1,573,200

111 more, such bleaching or decolorization as could be obtained by the use of the bleaching agents mentioned above, or their equivalents, ordinarily required from about 24 to 6 about 72 hours for the accomplishment of the poor and unsatisfactory results obtainable by their use.

By means of the present invention we are enabled to decolorize or bleach dark colored fur skins or the like without weakening or destroying the leather of the skins and without weakening or impairing the natural texture and strength of the hair. Skins bleached or decolorized in accordance with the principles of the present invention may thereafter be very readily and expeditiously dyed the same colors, light or otherwise, as can at present be applied with success only to natural white or light colored furs. Furthermore, the entire combined operation of bleaching or decolorizing the skins and thereafter dyeing them in accordance with the principles of the present invention requires only as much, or even less, time as the ordinary fur dyeing process. Furthermore, the resultant bleached or decolorized skins and the subsequently dyed skins are characterized by the leather of such skins coming out of the process in sound condition as to strength and texture, and by the hair likewise coming out of the process in sound condition as to strength, texture and lustre. In fact, furs treated in accordance with the present invention come out of the process, after the combined bleaching or decolorizing and subsequent dyeing operations, affected less, or only as much, as furs which have been merely dyed by the dyeing methods hitherto customarily employed.

40 We have discovered that by treating the fur skins or the like which are to be bleached or decolorized, prior to the bleaching or decolorizing step, with a protective agent, generally a reducing compound, preferably of mineral origin, such as a ferrous compound, for example, ferrous sulphate, in some way, the reasons for which are at present not clearly understood by us, such protective agent, while permitting the bleaching or decolorizing action to proceed under the action of the bleaching agent with remarkable rapidity, protects the leather and the hair of the fur skins or the like from any destructive or weakening effect of the bleaching agent.

45 For instance, while decolorization or bleaching of the fur skins or the like takes place under the action of the bleaching agent, for example, hydrogen peroxide, within as short a time as from about 1 to about 4 hours, instead of the 24 to 72 hours hitherto required for bleaching fur skins by the methods hitherto in use and employing such a bleaching agent, the leather and hair

50 of the skin bleached in accordance with the

principles of the present invention will be found to be in perfect condition, with their strength, texture and lustre unimpaired. While we do not wish to be limited to any particular theory or explanation as to why this remarkable, unexpected and commercially valuable result is obtained, our present explanation is that the presence in the fibres of the fur skin or the like of the mineral reducing agent, or its equivalent, locally prevents too violent action of the oxidizing or equivalent bleaching agent, such as the hydrogen peroxide referred to above, but without preventing the bleaching or decolorizing action from being carried out in the desired manner. In fact, the presence of the protective agent, such as the ferrous compound referred to, or its equivalent, not only protects the leather and the hair of the fur skins or the like from destructive or weakening action, but actually accelerates the desired decolorizing or bleaching action so that the bleaching operation takes only from about one (1) to about four (4) hours in place of the 24 to 72 hours hitherto required for the imperfect or even destructive bleaching as hitherto practiced.

55 Since the protective agent and bleach accelerator, in accordance with the principles of the present invention, generally comprises a reducing agent or compound, preferably of mineral origin, such as a ferrous compound, for example, ferrous sulphate, which would tend to be oxidized more or less readily on exposure to the air, we prefer to add to the protective agent, preferably before the same is applied to the fur skin or the like, prior to the bleaching or decolorizing operation, a stabilizing agent. The purpose of the stabilizing agent is to stabilize the protective agent and to prevent too rapid oxidation or deterioration of the same. Where, as is preferred, ferrous sulphate is used as the protective agent, we prefer to use for the stabilizing agent ammonium chloride. The fur skins or the like, after having been treated with a solution of the protective compound, which may or may not contain dissolved therein the stabilizing agent, are thereafter subjected to the bleaching operation, after which it may be dyed in any of the light or other shades such as can at the present time be produced only by dyeing natural white or other light colored skins.

60 The following is a specific example of one mode of applying the method of the present invention, it being understood, however, that the following description is given merely by way of illustration and that the process is not limited to the specific details of the following illustrative example:

65 Brown mouttons are washed or "killed" in an alkaline solution, for example, a solu-

tion of sodium carbonate. This washing operation ordinarily requires from about 2 to about 3 hours. The washed or "killed" skins are then rinsed and thoroughly hydro-extracted. The skins are then immersed in a solution of the protective agent, such as in a solution of ferrous sulphate, and there allowed to remain over night. While the strength of the ferrous sulphate solution or 10 its equivalent may vary within considerable limits, we prefer to use an aqueous solution of ferrous sulphate of a strength of from about 0.5 to about 5.0 per cent of the solid crystallized ferrous sulphate, by weight. 15 Such a solution may or may not contain the stabilizing agent. If a stabilizing agent, such as ammonium chloride, is used, we prefer to use it in an amount approximately equal to the amount of ferrous sulphate used 20 and equalling from about 0.5 to about 5.0 per cent of ammonium chloride, by weight.

The fur skins or the like, after having been soaked for from about 8 to about 12 hours in the solution of the protective agent, 25 with or without the addition of the stabilizing agent, are then rinsed and hydro-extracted. The treatment apparently impregnates or fills the voids and interstices of the fibres with the solution of protective agent. 30 The fur skins thus treated are now immersed in a solution of hydrogen peroxide or equivalent bleaching agent. However, in place of hydrogen peroxide, we may use other bleaching agents, particularly sodium 35 peroxide or sodium perborate, which yield hydrogen peroxide in solution in the presence of certain liberating agents, generally of an acid character. The amount of hydrogen peroxide used may vary from about five 40 (5.0) to about one hundred (100.0) per cent by volume of a three (3.0) per cent solution of hydrogen peroxide. We prefer that the temperature at which the bleaching or decolorizing operation is carried out shall 45 be between 60° and 100° F.

The skins are subjected to the action of the bleaching or decolorizing agent until they have been sufficiently decolorized. The bleached or decolorized skins are then rinsed 50 and can, if desired, be dyed directly in accordance with any of the well known or desirable processes employed for dyeing furs or the like. We may, however, subject the bleached or decolorized skins to the usual 55 dyeing operations of washing and mordanting, and then dyeing the washed and mordanted skins in accordance with the practice hitherto generally employed for dyeing furs.

60 It may here be stated, especially in connection with the foregoing specific example of applying the method of the present invention, that the original washing or "killing" operation to which the fur skin or the like is preferably subjected prior to its treat-

ment with the solution of the protective agent, may be combined as a single step with the treatment of the fur skin or the like with the protective agent, as by having the protective agent and also, if desired, the 70 stabilizing agent, present in the alkaline or other solution used for washing or "killing" the fur skins or the like. Or else, if desired, the washing or "killing" operation may be altogether omitted and satisfactory results 75 still obtained. It may here also be stated that a metallic salt or salts may be added to the solution of the protective agent, with or without the stabilizing agent, provided such metallic salt or salts are compatible with the 80 ferrous sulphate or equivalent protective agent. In such a case the decolorizing or bleaching process proceeds in exactly the same way as before, while the additional salt or salts act as a mordant for the subsequent 85 dyeing process where a mordant is desired to be employed.

Where the fur is preliminarily washed or "killed", as with a solution of an alkaline substance, the nature of the fur will determine the nature and strength of the particular alkaline substance, or its equivalent, to be used in the washing or "killing" operation. It may here further be stated that while, in accordance with our experience up to the present time, the foregoing process may be successfully applied to all dark colored furs, the concentration of the reagents employed and the length of time for subjecting the fur skins or the like to the various operations will depend very largely upon the nature of the skins or the like being treated, the factors of temperatures, concentrations, lengths of time of treatment, and the like, for any particular kind of fur, being readily determined by trial and experiment.

The advantages of the foregoing process are numerous and of great practical importance, and may be briefly summarized as 110 follows: In the first place, the process enables dark colored fur skins or the like to be bleached or decolorized to a white or very light color without destroying or even weakening the leather of the skins, and without impairing the strength, texture or lustre of the hair of such skins. The process is at the same time very simple, convenient, and economical to practice, and while enabling the 115 desired decolorizing or bleaching operation to be conducted safely and with due regard to the strength and texture of the final product, serves in a simple and inexplicable way to accelerate the bleaching or decolorizing operation.

120 By means of the present invention we are enabled to accomplish the tremendously important and commercially invaluable result of bleaching or decolorizing the comparatively cheap, dark colored fur skins or the 130

## TREATMENT &amp; CHEMICAL MODIFICATION OF TEXTILES &amp; FIBERS, 1,573,200

111

like to a white or very light color, without destroying or impairing the strength and fineness of texture of the fur skin or the like, thus enabling the cheaper dark furs to be successfully bleached and decolorized, and thereafter as successfully dyed in all the light colors hitherto obtainable only by dyeing natural white or light colored skins. The resulting bleached or decolorized, and subsequently dyed, fur skin or the like, which is more fully described and which is claimed in our copending application referred to above, is characterized by its remarkably fine texture and lustre, and by having practically all of the strength of the unbleached skin. In fact, skins bleached or decolorized, and subsequently dyed, in accordance with the principles of the present invention will be found to have lost less of their strength, texture and lustre, than skins subjected merely to the dyeing operation as hitherto practiced. So fine is the product obtained by the practice of the present invention, and so closely does it resemble the skin obtained by dyeing the natural white or light colored fur, that only an expert, if even an expert, can distinguish the one from the other, while the bleached and light dyed skin fetches almost the same high price that the natural white or light colored skin fetches in the present market.

It may here be stated that in addition to the mineral protective agent, such as the ferrous sulphate, with or without the addition of the stabilizing agent, the solution for giving the fur skins or the like their protective treatment for the subsequent bleaching operation may contain other compatible metal salts, as well as suitable protective colloids, such as glue, gelatin, or the like, generally in relatively small amounts. It may here also be stated that the method described above may be applied with almost equal success in the treatment of skins which have already been dyed, either a dark or a light color, especially skins which have been unsatisfactorily dyed or spoiled in the dyeing operation, such as skins which have been dyed by the use of a mordant consisting of a ferrous compound, such as ferrous sulphate, or an equivalent substance, thus producing from the previously dyed skins the superior product described above.

55 What we claim as our invention is:

1. The method of bleaching fur skins and the like, which comprises treating the fibres with an oxidizing agent in the presence of a protecting agent comprising a reducing compound.
2. The method of bleaching fur skins and the like, which comprises treating the same with an oxidizing agent in the presence of an accelerator comprising a mineral reducing compound.
3. The method of bleaching fur skins and the like, which comprises treating the same with a solution of hydrogen peroxide in the presence of an accelerator comprising a mineral reducing compound. 70

4. The method of bleaching fur skins and the like, which comprises treating the same with an oxidizing agent in the presence of an accelerator comprising a ferrous compound. 75

5. The method of bleaching fur skins and the like, which comprises treating the same with a solution of hydrogen peroxide in the presence of an accelerator comprising a ferrous compound. 80

6. The method of bleaching fur skins and the like, which comprises treating the same with a solution of a protecting agent to which has been added a stabilizing agent, and thereafter subjecting the articles so treated to the action of a bleaching agent. 85

7. The method of bleaching fur skins and the like, which comprises treating the same with a solution of a protecting agent to which has been added a stabilizing agent, and thereafter subjecting the articles so treated to the action of a solution of hydrogen peroxide. 90

8. The method of bleaching fur skins and the like, which comprises treating the same with a solution of a mineral reducing agent to which has been added a stabilizing agent, and thereafter subjecting the articles so treated to the action of a bleaching agent. 95

9. The method of bleaching fur skins and the like, which comprises treating the same with a solution of a ferrous compound, to which has been added a stabilizing agent, and thereafter subjecting the articles so treated to the action of a bleaching agent. 100

10. The method of bleaching fur skins and the like, which comprises treating the same with a solution of a ferrous compound, and thereafter subjecting the article so treated to the action of a bleaching agent. 105

11. The method of bleaching fur skins and the like, which comprises treating the same with a solution of a protecting agent to which has been added ammonium chloride, and thereafter subjecting the articles so treated to the action of a solution of hydrogen peroxide. 110

12. The method of bleaching fur skins and the like, which comprises treating the same with a solution of a ferrous compound to which has been added ammonium chloride, and thereafter subjecting the article so treated to the action of a bleaching agent. 120

13. The method of bleaching fur skins and the like, which comprises treating the same with a solution of a mineral reducing agent to which has been added ammonium chloride, and thereafter subjecting the articles so treated to the action of a bleaching agent. 125

14. The method of bleaching fur skins and the like, which comprises treating the same with a solution of a protecting agent to which has been added ammonium chloride, and thereafter subjecting the articles so treated to the action of a bleaching agent. 45
15. The method of dyeing animal fibres, particularly fur skins and the like, which comprises bleaching the same in the presence of a fibre-protecting bleach accelerator comprising a ferrous compound, and thereafter dyeing the product so bleached. 50
16. The method of dyeing animal fibres, particularly fur skins and the like, which comprises bleaching the same with a solution of hydrogen peroxide in the presence of a fibre-protecting bleach accelerator comprising ferrous sulphate, and thereafter dyeing the product so bleached. 55
- 20 17. The method of dyeing animal fibres, particularly fur skins and the like, which comprises bleaching the same in the presence of a fibre-protecting bleach accelerator comprising a ferrous compound to which has been added a stabilizing agent, and thereafter dyeing the product so bleached. 60
- 30 18. The method of dyeing animal fibres, particularly fur skins and the like, which comprises bleaching the same with a solution of hydrogen peroxide in the presence of a fibre-protecting bleach accelerator comprising ferrous sulphate to which has been added ammonium chloride, and thereafter dyeing the product so bleached. 65
- 35 19. The method of dyeing animal fibres, particularly fur skins and the like, which comprises bleaching such fibres in the presence of a fibre-protecting agent comprising a reducing substance, and thereafter dyeing the bleached product. 70
- 40
20. The method of dyeing animal fibres, particularly fur skins and the like, which comprises bleaching such fibres in the presence of a fibre-protecting agent comprising a ferrous compound, and thereafter dyeing 45 the bleached product.
21. The method of dyeing animal fibres, particularly fur skins and the like, which comprises bleaching such fibres in the presence of a fibre-protecting agent comprising 50 ferrous sulphate, and thereafter dyeing the bleached product.
22. The method of dyeing animal fibres, particularly fur skins and the like, which comprises bleaching such fibres with a solution of hydrogen peroxide in the presence of a fibre-protecting agent comprising a reducing substance, and thereafter dyeing the bleached product. 55
23. The method of dyeing animal fibres, particularly fur skins and the like, which comprises bleaching such fibres with a solution of hydrogen peroxide in the presence of a fibre-protecting agent comprising a ferrous compound, and thereafter dyeing 60 the bleached product.
24. The method of dyeing animal fibres, particularly fur skins and the like, which comprises bleaching such fibres with a solution of hydrogen peroxide in the presence of a fibre-protecting agent comprising ferrous sulphate, and thereafter dyeing the bleached product. 70

In testimony whereof, we have signed our names to this specification this 23rd day of 75 April, 1924.

HYMAN STEIN.  
WILLIAM E. AUSTIN.  
IRVING LIEBOWITZ.